

**1**

2,856,371

**METHOD FOR STORING HYDROSOLS IN A DRY REUSABLE STATE**

John W. Gates, Jr., John R. Dann, and Bernard D. Illingsworth, Rochester, N. Y., assignors to Eastman Kodak Company, Rochester, N. Y., a corporation of New Jersey

No Drawing. Application December 14, 1953  
Serial No. 398,235

5 Claims. (Cl. 260—8)

This invention relates to a method for the dry storage of polymeric hydrosols by which those dry materials may be readily redispersed in aqueous liquids.

There are many polymeric hydrosols which are of value in compositions such as coating compositions and the like. However, it has been a characteristic of those hydrosols heretofore that when the liquid content thereof is removed the resulting solid material has not been capable of redispersion. Consequently, when shipping or storage of those materials is indicated the bulkiness of the hydrosols creates a problem which would be avoided if only the solid portion of those hydrosols could be handled.

One object of our invention is to provide a method for converting polymeric hydrosols to a dry form in a state in which redispersion may be readily accomplished. Other objects of our invention will appear herein.

We have found that polymeric hydrosols may be safely dried down to a form which admits of redispersion if there is added to the hydrosol an amount of gelatin at least equal to the amount of the hydrosols, based on the dry weight of each, prior to the drying operation. The product so obtained can be stored for long periods of time and when the material is desired in dispersed form the dried materials will readily admit of dispersion in water or some other liquid in which water predominates.

The method of carrying out our process involves the dispersing of the polymeric hydrosols made up of discrete dispersed particles in a gelatin solution in a proportion that the gelatin constitutes at least equal parts to the hydrosol figured in terms of dry weight. The composition thus prepared may be set by chilling and the drying may then be accomplished in any manner conventional to the drying of gelatin. The proportion of gelatin to hydrosol, dry weight, should be within the range of 9:1 to 1:1. If an amount of gelatin much below this range is employed the hydrosol is "denatured" by drying, that is, redispersion will not take place. It seems as if the gelatin forms a protective coating for the particles of the hydrosol and preserves that dry material in such a form that the water readily disperses those particles.

In the carrying out of our invention there is no need to make any radical adjustment in the condition of the gelatin as the preparation of these dispersions at a pH of 6, which is the pH at which gelatin dispersions are generally obtained, is suitable. We have also found that the preparation of the dispersions at 10% gelatin concentration works satisfactorily in the carrying out of our invention although, of course, other concentrations can be employed and the desired effect will be obtained. After the composition of gelatin and the polymeric hydrosol has been prepared, the mixture of gelatin and hydrosol can be conveniently converted to the form of noodles or slices such as by chilling which sets the gelatin. These particles may be washed with cold water prior to drying and also any water soluble impurities which might be present may be removed by such a wash-

**2**

ing operation. The hydrosols thus prepared by this procedure are of high quality. Also we have found that the photographic quality of the hydrosols is not adversely affected by preparing in dry form in accordance with our invention. The dry compositions thus obtained may be stored for long periods or may be redispersed after holding for any convenient time such as where shipping of the hydrosol material is desired. The polymeric hydrosols which may be handled or stored in accordance with our invention may be any of the latices which are well known as useful for coating operations, may be a polymeric hydrosol such as the type described and claimed in U. S. applications Serial Nos. 398,234 and 398,236 of Gates and Fowler and Gates, Dann, and Illingsworth, respectively, which applications are being filed of even date, or the polymer may be a polymeric hydrosol of the type described and claimed in U. S. applications Serial Nos. 272,709 and 336,431 of Fowler, filed February 20, 1952, and February 11, 1953, respectively. Any other polymeric hydrosols of a similar nature may be handled and stored as desired in accordance with our invention. The following examples illustrate our invention:

*Example 1*

25 A hydrosol was prepared having a 20% solid content in the preparation of which sodium lauryl sulfate and a mixture of 59 parts of n-butylacrylate, 25 parts of acrylonitrile and 16 parts of 5% maleated glue was employed. These were mixed in water so as to form a 20% solids aqueous dispersion of these materials. This dispersion was mixed with a 20% aqueous dispersion of gelatin in the ratios of dry weight of gelatin to dry weight of hydrosol of 9:1, 7:3, 1:1. The mixtures were chilled, sliced, washed, when necessary, and dried in the conventional manner. The resulting material was obtained in the form of flakes. To redispense the dry flakes they were soaked in water at 25° C. for 1/2 hour and then warming to 50° C. accompanied by stirring. The mixtures were found to readily redispense. The hydrosol 40 was prepared in accordance with the procedure described in the Gates and Fowler application filed of even date herewith.

*Example 2*

45 A hydrosol was prepared by an emulsion polymerization as described in our application filed of even date using sodium lauryl sulfate as the micell-forming surface active agent. The reaction mass was composed of 49 parts of n-butylacrylate, 21 parts of acrylonitrile and 30 parts of glue, these materials being present in a proportion of 20% of the mass. The hydrosol thus prepared was mixed with gelatin in ratios of 9:1, 7:3 and 1:1, dry weight, gelatin to hydrosol. It was found that these mixtures after drying are susceptible to redispersion in water.

*Example 3*

55 A hydrosol having a 20% solids content was prepared of a mixture of 49 parts of n-butylacrylate, 21 parts of styrene, and 30 parts of glue by an emulsion polymerization as described in our application filed of even date with sodium lauryl sulfate employed as the micell-forming surface active agent. This preparation follows the teachings of the Gates and Fowler application referred to above. The hydrosol was mixed with gelatin in the ratios of 1:9, 3:7 and 1:1, dry weight, and the mixtures 60 were dried. It was found that these dry compositions can be readily redispersed in water whenever desired.

*Example 4*

70 A hydrosol was prepared by the emulsion polymerization of a mixture of 84 parts of n-butylacrylate and 16 parts of 5% maleated glue so as to form a hydrosol hav-

ing a 20% solids content. The hydrosol thus prepared was mixed with gelatin in ratios of 9:1, 7:3, 1:1, the ratios in every case being by dry weight. The compositions thus obtained were dried and were found to be readily susceptible to redispersion in water when such a dispersion is desired.

*Example 5*

A hydrosol was prepared by the emulsion polymerization of a mixture of 49 parts of n-butylacrylate, 21 parts of styrene and 30 parts of 5% maleated glue at a 10% solids content with sodium lauryl sulfate. The hydrosol thus prepared was mixed with gelatin in the ratios of gelatin to hydrosol, dry weight, of 4:1, 7:3, 3:2, and 1:1 in the same manner as described in Example 1. It was found that the dried materials would redisperse in water when the preparation of a dispersion was desired.

*Example 6*

A polymeric hydrosol was prepared of a mixture consisting of 49 parts of n-butylacrylate, 21 parts of styrene, and 30 parts of 5% maleated glue using a 10% solids concentration. The hydrosol thus prepared was mixed with gelatin and treated as described in Example 1, the ratios of gelatin to hydrosol by dry weight being as follows: 4:1, 7:3, 3:2, 1:1. The dried material was susceptible to redispersion in water when the preparation of a dispersion thereof was desired.

*Example 7*

A hydrosol was prepared by the emulsion polymerization of a mixture of 20% solids content of 42 parts of n-butylacrylate, 42 parts of styrene, and 16 parts of methacrylamide in the presence of a surface active agent, this emulsion polymerization having been carried out as taught in U. S. application Ser. No. 272,709 of William F. Fowler, Jr. The hydrosol thus prepared was mixed with gelatin in ratios of gelatin to hydrosol, by dry weight, of 9:1, 7:3 and 1:1 and the mixtures thus obtained were dried in the manner taught in Example 1. The dried materials were found to be readily susceptible to redispersion in water.

*Example 8*

A styrene-butadiene latex of 20% solids content was mixed with gelatin in the ratios of 9:1, 7:3, and 1:1 gelatin to latex by dry weight. These mixtures were dried in the manner taught in Example 1. The dried materials were found to be readily susceptible to redispersion in water.

We claim:

1. A method of handling polymeric hydrosols which comprises mixing 1 part of a polymeric hydrosol resulting from an emulsion copolymerization in which one of the monomers employed therein was selected from the group consisting of the alkyl acrylates, the alkyl methacrylates, butadiene, isoprene and chloroprene, and in which the other monomer is at least one of the group consisting of

styrene, acrylonitrile and methacrylamide, with 1-9 parts of an aqueous solution of only gelatin, all by dry weight, converting the mass to solid form by chilling, dividing the mass into small independent units and substantially completely drying those units and later redispersing the units in water.

2. A method of handling polymeric hydrosols which comprises mixing 1 part of a polymeric hydrosol resulting from the emulsion copolymerization of a mixture of an alkyl acrylate, acrylonitrile, and a gelatin compound selected from the group consisting of gelatin and the unsaturated acid derivatives of gelatin with 1-9 parts of an aqueous solution of only gelatin, all by dry weight, converting the mass to solid form by chilling, dividing the mass into small independent units and substantially completely drying those units and later redispersing the units in water.

3. A method of handling polymeric hydrosols which comprises mixing 1 part of a polymeric hydrosol resulting from the emulsion copolymerization of a mixture of an alkyl acrylate, styrene, and a gelatin compound selected from the group consisting of gelatin and the unsaturated acid derivatives of gelatin with 1-9 parts of an aqueous solution of only gelatin, all by dry weight, converting the mass to solid form by chilling, dividing the mass into small independent units and substantially drying those units and later redispersing the units in water.

4. A method of handling polymeric hydrosols which comprises mixing 1 part of a polymeric hydrosol resulting from the emulsion copolymerization of an alkyl acrylate, styrene, and methacrylamide with 1-9 parts of an aqueous solution of only gelatin, all by dry weight, converting the mass to solid form by chilling, dividing the mass into small independent units and substantially completely drying those units and later redispersing the units in water.

5. A method of handling polymeric hydrosols which comprises mixing 1 part of styrene butadiene copolymer latex compatible with gelatin with 1-9 parts of an aqueous solution of only gelatin, all by dry weight, converting the mass to solid form by chilling, dividing the mass into small independent units and substantially completely drying those units and later redispersing the units in water.

References Cited in the file of this patent

UNITED STATES PATENTS

|    |           |                    |               |
|----|-----------|--------------------|---------------|
| 45 | 1,762,494 | Wescott            | June 10, 1930 |
|    | 2,019,055 | Noble              | Oct. 29, 1935 |
|    | 2,500,028 | Griggs et al.      | Mar. 7, 1950  |
| 50 | 2,548,520 | Damschroder et al. | Apr. 10, 1951 |
|    | 2,739,137 | Fowler             | Mar. 20, 1956 |

FOREIGN PATENTS

|    |         |               |               |
|----|---------|---------------|---------------|
| 55 | 213,886 | Great Britain | June 19, 1924 |
|----|---------|---------------|---------------|

OTHER REFERENCES

Noble: "Latex in Industry," published by Polmerton Publishing Co., September 1953, 2nd edition, page 148.